# EUROPEAN PATENT SPECIFICATION

(11) **EP 0 565 363 B1**
(45) Date of publication and mention of the grant of the patent: **26.06.1996**
(21) Application number: 93302736.9
(22) Date of filing: 07.04.1993
(51) Int. Cl.: H01F 1/053, H01F 41/02

(54) **Method for producing anisotropic rare earth magnet**
Herstellungsverfahren für einen anisotropen Seltenerd-Magneten
Méthode de production d'un aimant de terre rare anisotrope

(30) Priority: 09.04.1992 JP 116821/92
(43) Date of publication of application: 13.10.1993
(73) Proprietor: DAIDO TOKUSHUKO KABUSHIKI KAISHA, Naka-ku Nagoya-city Aichi-prefecture (JP)
(72) Inventor: Kasai, Yasuaki, No. 401 Glorious Narumi, Nagoya-city, Aichi-pref. (JP); Yoshikawa, Norio, No. 303 Yoshizawa Bldg., Nagoya-city, Aich-pref. (JP); Yamada, Hiyoshi, Iwakura-city, Aichi-pref. (JP)
(74) Representative: Jenkins, Peter David

(56) References cited:
- EP-A- 0 334 478
- EP-A- 0 392 799
- PATENT ABSTRACTS OF JAPAN vol. 15, no. 387 (E-1117)30 September 1991 & JP-31 55 107
- PATENT ABSTRACTS OF JAPAN vol. 14, no. 493 (E-0995)26 October 1990 & JP-22 03 510

## Description

This invention relates to a method for producing an anisotropic rare earth magnet, and in particular to a method for extruding a compacted material in order to obtain a better yield of the anisotropic rare earth magnet excellent in magnetic properties.

Rare earth magnets represented by R-Fe-B (R is shown on behalf rare earth metals of lanthanum series) are provided in two types as mentioned hereunder:
(a) a sintered magnet which is made into an anisotropic magnet through a process of casting the molten base alloy into an ingot, pulverizing the ingot into super fine powder, pressing the powder in a magnetic field and sintering it, and
(b) a super-quenched magnet which is given with magnetic anisotropy through a process of making a thin flake by cooling the molten base alloy super-rapidly, molding a compacted material with magnetic isotropy by compressing coarse grained powder of the thin flake of the base alloy and deforming the compacted material plastically.

The anisotropic rare earth magnets obtained through the aforementioned processes have excellent magnetic properties, therefore it is very useful to apply these magnets to small-sized electric motors used for various automated apparatuses in order to make the motors lighter and smaller.

EP-A-0334478 discloses a method of increasing the volume fraction of magnetically-aligned material in rare earth (RE), iron, boron type anisotropic permanently magnetic material. This method includes forming an adaptively-shaped, fully-dense, substantially magnetically-isotropic preform from relatively coarse powder particles of melt-spun alloy containing a very fine-grain RE₂Fe₁₄B phase. The preform is heated and die-upset to provide uniformity of strain in the preform as it is conformed to the die walls, thereby causing an increased percentage of the crystallites in the preform to be oriented along crystographically-preferred magnetic axis which increases the energy product of a resultant magnet formed therefrom.

It is desirable to make ring-shaped magnets with magnetic anisotropy in the radial direction in order to apply the anisotropic rare earth magnets in motors. However, there is a problem since it is difficult to apply a magnetic field in the radial direction at the time of molding the powder in a magnetic field in the case of the aforementioned sintered magnet.

In the case of the super-quenched magnet, it is possible to give the magnetic anisotropy in the utmost limit even for the ring-shaped magnet because the magnetic anisotropy is given by the plastic deformation without forming in the magnetic field.

As a method for giving the magnetic anisotropy by the plastic deformation, heretofore, it is taken to extrude the compact material with magnetic isotropy formed in a hollow or solid circular plate-like shape, as disclosed in U.S. Patent No. 4,963,320, for example.

An example of the extruding is shown in Figure 4. In the figure, numeral 100 is a cylindrical die formed in a thick-walled cylindrical shape, numeral 102 is a bottom die forming a bottom part of a mold.

Numeral 104 is a core punch and numeral 106 is a sleeve punch disposed movably in a molding cavity 108 formed between the core punch 104 and the cylindrical die 100. The mold is constructed from the cylindrical die 100, the bottom die 102, the core punch 104 and the sleeve punch 106.

The bottom die 102 is provided with a hollow part 112 to receive a slender part 110 of the core punch 104.

In this method for giving anisotropy, a hollow circular plate-like (ring) shaped compacted material 114 is charged into the cylindrical die 100 of the mold, subsequently the compacted material 114 is extruded backwardly by pressing the core punch 104 into the compacted material 114 at the same time of compressing a free surface of the compacted material 114 fronting on the molding cavity 108 with the sleeve punch 106 moving back according as the progress of the extruding, thereby making the compacted material 114 anisotropic in the radial direction at the same time of forming the compacted material 114 into a hollow cylindrical magnet material.

However, in the aforementioned extruding method, magnetic properties at the upper end portion of the cylindrical magnet material shown with symbol A in Figure 4B are not so good as compared with, for example, a portion shown with symbol B in this figure, and there is a problem since it is not possible to use the upper end portion A practically.

This invention is made in order to solve the aforementioned problem of the prior art.

The present invention provides a method of producing an anisotropic rare earth magnet, which comprises charging a compacted rare earth magnet material into a cylindrical die of a mold, pressing the compacted material with a punch and plastically deforming the compacted material into a magnet having magnetic anisotropy and a ring-shaped section by extruding said compacted material into a molding cavity formed between the punch and the cylindrical die of the mold, characterised in that said compacted material is formed with an outer peripheral part which faces said molding cavity and a raised central part which contacts an end face of the punch.

The reason why the upper end portion A of the cylindrical magnet material is not so good in the magnetic properties is supposed that the portion A, being a part extruded into the molding cavity 108 at the beginning of the extruding, is extruded in the molding cavity 108 without plastic-deforming sufficiently in the radial direction, so that the degree of deformation at the portion A is low as compared with the other portion of the cylindrical magnet material.

According to the preferred embodiment of this invention, the compacted material of the rare earth magnet is formed in the shape having difference in level between the center part to be in contact with the end face of the punch and the outer peripheral part to be faced with the molding cavity formed between the punch and the cylindrical die of the mold, and extruded. Therefore, it is possible to deform plastically even the portion extruded in the molding cavity at the beginning of the extruding sufficiently.

Accordingly, in a case where the compacted material is extruded into the hollow cylindrical shaped magnet material, it is possible to improve the magnetic properties at the end portion of the cylindrical magnet material, and it is possible to increase yield rate of the expensive rare earth magnet since the end portion also can be used similarly to the other portion of the cylindrical magnet material.

An embodiment of the present invention will now be described by way of example only with reference to the accompanying drawings in which:
Figures 1A, 1B and 1C are sectional views illustrating the extruding method of the compacted material in an embodiment of the method for producing the rare earth magnet according to this invention;
Figure 2 is a sectional view illustrating a shape of the compacted material of the rare earth magnet used in the embodiment of the method according to this invention;
Figure 3 is a sectional view illustrating a shape of the compacted material used in another embodiment of the method according to this invention; and
Figures 4A and 4B are sectional views illustrating the conventional extruding method of the compacted material.

An embodiment of the method according to this invention will be described below on basis of Figure 1 to Figure 2.

Figure 1 shows an example of a case where the compacted material of the rare earth magnet is extruded backwardly, numeral 10 in the drawing denotes a cylindrical die and numeral 12 denotes a bottom die disposed detachably in the bottom part of the cylindrical die 10. Numeral 14 is a core punch, and numeral 16 is a sleeve punch disposed in a molding cavity 18 formed between the core punch 14 and the cylindrical die 10 so as to move backwardly according as extruding of the compacted material. A mold 13 is constructed from the cylindrical die 10, the bottom die 12, the core punch 14 and the sleeve punch 16.

Additionally, the core punch 14 is provided with a slender part 22 facing downward in the drawing, and the bottom die 12 is formed with a hollow part 24 in a position corresponding to the slender part 22.

In the method according to this embodiment, first of all, a compacted material 20 of the rare earth magnet is charged in the cylindrical die 10 of the mold 13 as shown Figure 1A, and the compacted material 20 is heated at a predetermined temperature together with the mold 13. The mold 13 and the compacted material 20 are so designed as to be housed in a closed chamber, and the extruding of the compacted material 20 will be carried out in a non-oxidative atmosphere by evacuating the closed chamber to a pressure lower than 1 Torr or replacing the atmosphere of the closed chamber with inactive gases such as argon.

The compacted material 20 is formed in a hollow circular plate-like shape as a whole; an inner peripheral part 26 being made higher than an outer peripheral part 28 by projecting the center portion in the axial direction.

Namely, the compacted material 20 is formed with difference in level between a part to be in contact with a pressing face at the end of the core punch 14 and a part to be faced with the molding cavity 18.

After charging the compacted material 20 in the mold 13, the core punch 14 and the sleeve punch 16 disposed coaxially are inserted in the cylindrical die 10 as shown in Figure 1B, and the end faces of the core punch 14 and the sleeve punch 16 are introduced into contact with the inner peripheral part 26 and the outer peripheral part 28 of the compacted material 20, respectively.

In this state, the compacted material 20 is deformed plastically and extruded backwardly by pressing the core punch 14 in the downward direction as shown in Figure 1C, thereby obtaining a cylindrical extrusion 25 (magnetic material).

In this way, the sleeve punch 16 compresses downwardly a free surface of the compacted material 20 extruded into the molding cavity 18 of the mold 13 and retreats as the extrusion of the compacted material 20 proceeds.

By performing the extrusion as the free surface of the compacted material 20 is compressed by the sleeve punch 16 in this manner, it is possible to prevent effectively the extrusion 25 from cracks.

The extrusion 25 extruded from the compacted material 20 as shown in Figure 1C is taken out of the mold 13 by moving the bottom die 12 relative to the cylindrical die 10, and is then magnetized in the radial direction according to well-known procedures. Whereby the cylindrical extrusion 25 becomes a rare earth magnet with radial anisotropy.

In the case where backward extrusion of the compacted material 20 is performed in accordance with the method of this embodiment, it is possible to deform plastically even the upper end portion of the cylindrical extrusion 25, that is the portion extruded into the molding cavity 18 at the beginning of the extruding, in the radial direction sufficiently. Therefore, excellent magnetic properties can be given to the aforemencioned portion.

The effect of the form and dimensions of the compacted material 20 on the magnetic propreties has been investigated. The following Example illustrates the results of such an investigation and is to be taken as non-limiting.

Namely, using powder of alloy consisting of 28 wt % of Nd, 2.5 wt % of Dy, 0.9 wt % of B, 5 wt % of Co, and balancing Fe as powder of magnetic material, five compacted materials 20 differing from each other in their dimensions L as shown in Figure 2 were made by compacting the powder in argon atmosphere at 800°C. Subsequently, each of the compacted materials 20 was extruded into the cylindrical extrusion 25 through the method shown in Figures 1A to 1C, and the cylindrical shaped anisotropic rare earth magnet was obtained by magnetizing the extrusion 25.

The results of the measurement of the magnetic properties of the obtained anisotropic rare earth magnet are shown in Table 1. The measured values in Table 1 denote the magnetic properties in the radial direction at the portion of upper 5mm length of the obtained cylindrical rare earth magnet.

**Table 1**

| L (mm) | Br (KG) | iIIc (KOe) | (BII) max (MGOe) |
|---|---|---|---|
| 0 | 9.2 | 17.3 | 17.0 |
| 2 | 10.3 | 16.7 | 24.2 |
| 4 | 11.2 | 16.1 | 30.1 |
| 6 | 11.5 | 15.8 | 31.8 |
| 8 | 11.6 | 15.8 | 32.1 |

From the experimental results shown in Table 1, it is clear that it is possible to give excellent magnetic properties even to the portion extruded into the molding cavity 18 at the beginning of the extrusion if extrusion is carried out using the compacted material 20 formed in a shape having the protruding inner peripheral part 26, and it is effective to improve the magnetic properties when the protruding height L of the inner peripheral part 26 of the compacted material 20 is not less than 4mm.

Although the invention has been described in its preferred embodiment, it is merely an example. This invention may be embodied in several forms modified according to knowledge of those skilled in the art without departing from the aim of this invention. For example, a solid compacted material 30 as shown in Figure 3 may be used as a substitute for the hollow-shaped compacted material 20 used in the aforementioned embodiment of this invention. Furthermore, the method in accordance with this invention may be also applied to a case in which the compacted material is formed into the extrusion by forward extruding.

## Claims

1. A method of producing an anisotropic rare earth magnet, which comprises charging a compacted rare earth magnet material (20) into a cylindrical die (10) of a mold (13), pressing the compacted material (20) with a punch (14,16) and plastically deforming the compacted material (20) into a magnet (25) having magnetic anisotropy and a ring-shaped section by extruding said compacted material (20) into a molding cavity (18) formed between the punch (14,16) and the cylindrical die (10) of the mold (13), characterised in that said compacted material (20) is formed with an outer peripheral part (28) which faces said molding cavity (18) and a raised central part (26) which contacts an end face of the punch (14).

2. A method of producing an anisotropic rare earth magnet as defined in claim 1, wherein said compacted material (20) is extruded at the same time as applying compressive force on a free surface thereof in the molding cavity (18).

3. A method of producing an anisotropic rare earth magnet as defined in claim 1 or claim 2, wherein said compacted material (20) is of a hollow and circular plate-like shape.

## Patentansprüche

1. Verfahren zum Herstellen eines anisotropen Seltenerdmagneten, welches umfaßt: Eingeben eines verdichteten Seltenerdmagnetmaterials (20) in einen zylindrischen Druckring (10) eines Formwerkzeugs (13), Pressen des verdichteten Materials (20) mit einem Stempel (14,16) und plastisches Verformen des verdichteten Materials (20) zu einem Magneten (25) mit magnetischer Anisotropie und einem ringförmigen Querschnitt durch Extrudieren des verdichteten Materials (20) in einen Formhohlraum (18), der zwischen dem Stempel (14,16) und dem zylindrischen Druckring (10) des Formwerkzeugs (13) gebildet ist, dadurch gekennzeichnet, daß das verdichtete Material (20) mit einem äußeren Umfangsteil (28), der zu dem Formhohlraum (18) hinweist, und einem erhabenen Mittelteil (26) ausgebildet wird, der mit einer Stirnfläche des Stempels (14) in Berührung steht.

2. Verfahren zum Herstellen eines anisotropen Seltenerdmagneten nach Anspruch 1, bei welchem das verdichtete Material (20) gleichzeitig mit der Anwendung einer Druckkraft auf eine freie Oberfläche desselben im Formhohlraum (18) extrudiert wird.

3. Verfahren zum Herstellen eines anisotropen Seltenerdmagneten nach Anspruch 1 oder 2, bei welchem das verdichtete Material (20) eine hohle und kreisförmige plattenartige Form besitzt.

## Revendications

1. Procédé de fabrication d'un aimant de terre rare anisotrope, qui comprend les opérations consistant à charger un matériau d'aimant de terre rare comprimé (20) dans une matrice cylindrique (10) d'un moule (13), presser le matériau comprimé (20) avec un poinçon (14, 16) et déformer plastiquement le matériau comprimé (20) en un aimant (25) avec une anisotropie magnétique et une section annulaire par extrusion dudit matériau comprimé (20) dans une cavité de moule (18) formée entre le poinçon (14, 16) et la matrice cylindrique (10) du moule (13), caractérisé en ce que ledit matériau comprimé (20) est doté d'une partie périphérique externe (28) qui donne sur ladite cavité de moule (18) et d'une partie centrale dressée (26) qui contacte une face d'extrémité du poinçon (14).

2. Procédé de fabrication d'un aimant de terre rare anisotrope selon la revendication 1, dans lequel ledit matériau comprimé (20) est extrudé en même temps qu'est appliquée une force de compression sur une surface libre du matériau dans la cavité de moule (18).

3. Procédé de fabrication d'un aimant de terre rare anisotrope selon la revendication 1 ou 2, dans lequel ledit matériau comprimé (20) est en forme de plaque circulaire et creuse.
